

June 5, 1956

V. BROWN

2,748,466

METHOD OF MAKING ENGINE HUB AND SHAFT UNIT

Filed Feb. 8, 1952



Inventor:  
Victor Brown

By *Hill, Hansen, Meoni, Clark & Simpson Atty's*

1

2,748,466

## METHOD OF MAKING ENGINE HUB AND SHAFT UNIT

Victor Brown, Elmhurst, Ill., assignor to Kropp Forge Company, Chicago, Ill., a corporation of Illinois

Application February 8, 1952, Serial No. 270,703

1 Claim. (Cl. 29—553)

This invention relates to an improved method of forming articles of forgeable material comprising a shaft having an integral enlarged portion at one end thereof, and more particularly to an improved method of forging a steel engine shaft having an integral hub or wheel at one end.

In the forging of articles such as steel axles, the general procedure involves the use of a stock piece having a thickness or diameter that is not only greater than the shaft but also greater than the journal or other special section which is integral with the shaft. The stock piece is first heated to a forging temperature and then placed between open dies in a forge for reducing or drawing down the stock piece. The forging ordinarily is begun at the middle of the stock piece, which may be rapidly reduced by heavy blows of the forge hammer; and the forging progresses toward a free end of the stock piece as the drawing down to shaft size is accomplished. By the use of different sized dies, the journal portion at the end of the shaft is then formed. Usually, also, it is necessary to smooth up the forging and bring the shaft to precisely the correct diameter by again going over the forging, using relatively light hammer strokes.

This process of drawing down is ordinarily adopted in preference to such forging operations as upsetting or welding, because it is open to no objection and it involves no risk or damage to the material, while it improves the metal by consolidating its "fibers." It is, of course, apparent that the greater the reduction in cross-sectional area of the piece, the greater the amount of work that must be expended during the drawing down operation. Also, the tediousness of the operation and the wear and tear on the dies are functions of the work that must be done. Moreover, excessive amounts of work done on a given stock piece may result in appreciable alteration of the characteristics of the metal.

In a typical engine shaft having an integral hub, or wheel the hub diameter is substantially greater than the shaft diameter and, in the production thereof by a procedure such as that just mentioned, a very great amount of work is required in reducing a stock piece from approximately the hub size to the shaft size. On the other hand, upset forging of a shaft size stock piece to form the hub at one end thereof would ordinarily involve such a substantial increase in the cross-sectional area of the piece at the hub portion that undesirable characteristics would be developed in the metal thereat, and an excessive amount of extra work would probably be required to realign the shaft after the upsetting operation.

The instant invention provides an improved method for forging such an engine shaft having an integral hub at one end whereby the benefits of the drawing down and upsetting operations are exploited by the use of a certain sequence of process steps, so as to reduce to a minimum the defective and undesirable possible results that might be obtained by the use of either of such operations alone.

It is, therefore, an important object of the instant in-

2

vention to provide an improved process of forming a shaft having an integral enlarged portion at one end thereof.

It is a further object of the instant invention to provide an improved process of forging an engine shaft having an integral hub at one end thereof, particularly if the hub is substantially greater in diameter than the shaft.

It is another object of the instant invention to provide an improved process of forging an engine shaft having an integral hub at one end, which comprises first upset drop-forging the hub at one end of a suitable stock piece and subsequently drawing down to shaft size the remainder of the forging.

It is still a further object of the instant invention to provide an improved process of forging an engine shaft having an integral hub at one end, which comprises upset drop-forging the hub at one end of a suitable stock piece, necking down to shaft size the upset forging immediately adjacent the hub, and drawing down to shaft size the remainder of the forging.

It is still another object of the instant invention to provide an improved process of forging an engine shaft having an integral hub and shaft nub at one end of the shaft, which comprises upset drop-forging a suitably cylindrical stock piece to accomplish simultaneously a two-three to one reduction in diameter of the piece to form the shaft nub, and a two-three to one expansion of the piece adjacent the nub to form the hub, trimming the forging, then necking down the forging to shaft size immediately adjacent the hub and simultaneously completing the hub formation, and next drawing down the forging to shaft size inwardly of the necking.

It is also an important feature of the instant invention to provide an improved forging process wherein the operational advantages of upset drop forging are obtained by carrying out such a step initially, using a piece suitably designed to reduce to a minimum the strains incurred during such operation, and subsequently employing a drawing down process, during which reheating of the piece may be employed to reduce any strains which might have been created during the upset drop forging operation.

Other objects, features and advantages of the present invention will become apparent to one skilled in the art from the following description of the embodiment illustrated in the accompanying drawings, in which:

Figure 1 is a side elevational view of an upset drop forging obtained by carrying out the initial upsetting operation of the invention, using a stock piece having approximately the dimensions shown in broken lines;

Figure 2 is an end elevational view of the upset drop forging of Fig. 1, taken from the hub end of the forging;

Figure 3 is a side elevational view of the aforementioned drop forging after the completion of a necking down operation according to the instant invention, also showing a fragmentary sectional view of the necking dies in position;

Figure 4 is a fragmentary sectional elevational view taken substantially along the line IV—IV of Fig. 3; and

Figure 5 is a side elevational view of an engine shaft having an integral hub at one end obtained by carrying out the process steps outlined in the foregoing figures.

As shown on the drawings:

In Figure 1, the broken lines designated by the reference numeral 10 indicate generally a generally cylindrical stock piece of suitably forgeable material, such as steel, which may be used in carrying out the initial upset drop forging operation of the invention. The metal stock piece 10 may have, for example, a diameter  $a$  of about 8 inches and a length  $b$  of about 30 inches. Prior to carrying out the first step in the process of the invention

the work piece 10 is heated to suitable forging temperatures in the manner well known in the art.

The work piece 10 is then positioned between a pair of upset drop forging dies, which define in cooperating position a space of the precise shape and contour of the upset forging designated generally by the reference numeral 11 in Figure 1.

The manner in which upset drop forging operations are carried out is generally well known in the art and need be described only briefly herein. In such an operation the stock piece 10 would, of course, be positioned vertically with, for example, the left end uppermost, instead of in the horizontal position shown in Figure 1. In a drop forging operation the cooperating dies (not shown) define the exact shape of the article to be forged. In this case the upper or hammer die (not shown) has a recess corresponding to the shape of the portion of the forging 11 at the left of the line X—X of Figure 1; and the lower or anvil die (not shown) has a recess corresponding to the shape of the portion of the forging 11 at the right of the line X—X. Upset forging or upsetting involves a reduction in the length of the stock piece by exertion thereagainst of opposed longitudinal forces, such as by the repeated dropping or hammering of the instant upper die against the left-hand end of the work piece 10 of Figure 1 while the right-hand end of the work piece is supported by the instant lower die, functioning as an anvil.

Any particular portion of the work piece which is to be changed in shape during the upsetting operation is heated to forging temperature prior to commencement of the operation. In the instant example here shown, the entire work piece 10 is preferably heated to forging temperature. After repeated hammering of the upper die against the piece 10 on the lower die, the work piece 10 assumes the form of the forging 11 and the upper and lower dies come face to face, causing the slight amount of excess metal to extrude as flash, outwardly in the plane defined or designated by the line X—X in Figure 1. The operation of trimming the flash, which is next carried out in the process of the invention, is carried out in the manner well known in the art and therefore need not be here described.

A particularly important advantage of the use of an initial drop forging operation in the instant invention, employing closed instead of open dies, resides in the fact that accurate die design may be used to control the precise total amount of metal to be employed in the process and thereby, for example, to determine the precise overall dimensions of the finally forged product that is obtained after carrying out the subsequent steps of the invention.

Referring again to Figure 1, it will be seen that at the extreme right end of the work piece 10 a shaft nub 12 is formed, having an average diameter  $c$  of perhaps 4 inches. The formation of the nub 12 thus involves a reduction in the diameter or thickness, which is preferably a reduction of about 2-3 to 1 in the practice of the invention. The nub is formed, of course, by driving the end portion of the work piece 10 into a suitably designed slightly tapering recess in the bottom die.

The shaft nub 12 is centrally mounted on an outwardly tapered boss-like face 13 of the engine hub 14. The boss-like face 13 of the engine hub 14 may thus be referred to as the end face thereof, as contrasted to the inward face 15 of the hub 14. It will also be appreciated that the end face 13 and the inward face 15 both taper outwardly toward the periphery of the hub 14, in conformance with the shape and contour of the recesses corresponding thereto in the lower and upper dies, respectively.

The engine hub 14 is formed during the upsetting operation by expansion of the diameter or thickness of the work piece to an approximate diameter  $d$  of perhaps 20 inches. The expansion thus obtained is preferably about 2-3 to 1 in the practice of the invention.

In the practice of the instant invention it has been

found preferable, in the upset drop forging operation, to effect an expansion also in the remaining portion 16 of the forging 11. As shown herein, the remaining portion 16 is positioned centrally on the inside face 15 of the hub 14 and has a slightly tapered generally cylindrical shape, with a rounded end 17 terminating the remaining portion 16 of the forging 11. The resulting average diameter  $e$  of the remaining portion 16 is perhaps 12 inches, and preferably the ratio of the hub diameter  $d$  to the diameter  $e$  is 5 to about 2-4 in the practice of the instant invention.

It has also been found that it is generally preferable in the practice of the invention to employ a ratio of the diameter  $e$  to the diameter  $a$  of about 5 to 3-4, and most preferably about 3 to 2. The reduction in the work piece length  $b$  to the overall drop forging length  $f$  in the instant example may be a reduction of 30 inches to about 24 inches, and is preferably a reduction of about 10 to about 9-7.

In the instant example, it has been found that an alteration of the dimensions of the work piece 10 during the conversion thereof to the upset drop forging 11 within the aforementioned approximate dimensional ranges is particularly suitable for the formation of the drop forging 11 so as to obtain an optimum combination of a minimum amount of work expenditure and a minimum amount of internal strain creation during the forging. Also, a minimum amount of overall material loss may be obtained thereby in carrying out the complete process of the invention, as will be pointed out hereinafter.

The next step involved in the instant process is the trimming of the flash from the drop forging 11 along the line X—X of Figure 1. As hereinbefore mentioned, such a procedure is well known in the art and the details thereof need not be set forth herein.

The next forging operation in the process of this invention is called a necking, or a necking down operation. Such process is carried out, as is indicated in Figures 3 and 4 of the drawings, by the use of upper and lower open swage-like dies 18 and 19, respectively, having mounted therein concentrically aligned, generally hemi-annularly shaped, inwardly tapering fuller-like die members 20 and 21, respectively.

As will be seen, each of the dies 18 and 19 has a first hemi-cylindrical recess 22 adapted to provide clearance between the dies 18 and 19 and the extreme periphery of the hub 14. Defining the inward peripheral portion of the surface of the recess 22 in each of the dies 18 and 19 is a semi-annular ledge 23, adapted to be positioned flush with the inward face 15 of the hub 14 for maintaining the proper cooperative position between the dies 18 and 19 and the hub 14.

The die members 20 and 21 in the upper and lower dies 18 and 19 respectively are positioned slightly inwardly of the ledge 23 in each die and cooperate with the ledge 23 to define a shoulder-like recess of generally outwardly tapered semi-annular shape in each of the dies 18 and 19. The die walls of that recess impart to the forging 11' (Fig. 3) a central concentric circular boss portion 24 mounted on the inward face 15 of the hub 14. It will thus be seen that the completion of the boss-like portion 24 of the hub 14 is accomplished simultaneously with the accomplishment of the necking down operation.

The necking down operation involves the cutting or fullering of an inwardly tapered annular groove in the forging 11'. By means of repeated hammering between the die members 20 and 21 the forging 11' is necked down to shaft size immediately adjacent the boss-like portion 24 of the hub 14. By "shaft size" is meant the approximate diameter  $g$  to which it is desired to ultimately draw down the remaining portion 16' of the forging 11' to complete the formation of the shaft 25, as designated in Figure 5. In the instant example, the diameter  $g$  is perhaps 5 inches, thereby resulting in a necking down reduction of

approximately 12 to 5 and preferably about 10 to about 3-6, in the practice of the invention.

As is best seen in Figure 4, the dies 18 and 19 mounting the cooperating die members 20 and 21, respectively, are open, as contrasted to closed (drop forging) dies. In other words, such dies are not shaped so as to conform precisely with the ultimate shape desired in the forging, particularly with respect to the annular groove or necking that is cut in the forging 11' adjacent the hub 14. The use of open dies in many instances, and particularly in the present instance, has been found to reduce appreciably the general wear and tear on the necking dies, as well as the internal strain creation during the necking operation.

It should also be noted that the dies 18 and 19 cooperate to define a pair of semi-cylindrical mating walls 26 inwardly (from the hub end) of the die members 20 and 21. The walls 26, when the dies 18 and 19 are matingly aligned, conform substantially to the shape and contour of the contiguous face portions of the remainder 16' of the forging 11'. The walls 26 may thus cooperate with the ledges 23 to check the alignment of the forging 11' at the end of the necking operation, when the walls 26 are brought into contact with the remainder 16' of the forging 11'.

It will also be appreciated that since the dies 18 and 19 are open dies, it would not be necessary to employ a corresponding die member 20 and 21 in both of such dies. The necking operation could be accomplished effectively by the use of a pair of dies wherein only one die contained the die member such as the die member 20 or 21. By rotation of the forging during the necking operation, the formation of the complete annular groove as well as the complete boss-like portion 24 of the hub 14 could be accomplished.

The next step in the process of the invention is the step of drawing down or reducing to shaft size the remaining portion 16' of the forging 11' of Figure 3 to obtain the shaft portion 25 shown in Figure 5. Drawing down is a well known forging operation which need not be described in detail herein. In general, the portion 16 is forged between generally hemi-cylindrically grooved swages (not shown). Preferably, the hammering down to shaft size is started at the portion of the forging near the necking and is worked on down the rest of the forging away from the hub 14.

The drawing down operation, as well as the prior trimming and necking down operations must, of course, be carried out upon forgeable metal heated to forging temperatures. In the instant example, it is usually desirable to reheat the forging at least once, and preferably twice, during the drawing down operation. In this respect, the instant invention provides a unique advantage in that all such reheating is carried out after the initial upsetting operation, so that any internal strains created during upsetting may have maximum opportunity to be released during the working as well as the reheating operation of the instant process, all of which are carried out subsequent to the upsetting operation. As is known, the drawing

down operations usually tend to reduce internal strain as well as to consolidate the "fibers" of the metal.

After the drawing down operation has been completed the resulting forging indicated generally by the reference numeral 26 in Figure 5 comprises an engine shaft having an integral hub at one end. The forged article 26 is cooled slowly to prevent flaking, and then checked for straightness. If straightening is required, preheating to about 1000° F. is usually necessary.

Next, the article is heated to about 1575° F. and maintained thereat in a continuous furnace for about five hours, and then oil-quenched. Immediately thereafter, the article 26 of the instant example is tempered in a continuous furnace at about 1100° F. for nine hours, to obtain 269 to 321.

Each of the forgings is, of course, serialized and given routine physical properties tests, including Brinell hardness. Also, various machining operations are usually carried out. For example, the shaft nub 12 would ordinarily be partially trimmed off and rounded down to remove the taper, and an annular recess would ordinarily be cut in the boss 24 on the hub 14. It will be appreciated that the instant forging process of the invention makes possible, by the use of an initial upsetting operation and a subsequent necking down operation, a minimum material loss and a minimum amount of machining in carrying out each of the aforementioned machining operations.

It will, of course, be understood that certain of the various foregoing details of structure and operation as herein set forth relate specifically to the instant example described herein, and various of such details may be varied through a wide range without departing from the principles of this invention; and it is not, therefore, the purpose to limit the patent granted hereon otherwise than necessitated by the scope of the appended claim.

I claim as my invention:

A process of forging a steel engine shaft having an integral hub and shaft nub at one end of the shaft, which comprises upset drop-forging a suitably cylindrical steel stock piece to accomplish simultaneously a 2-3 to 1 reduction in diameter of the piece to form the shaft nub and a 2-3 to 1 expansion in diameter of the piece adjacent the nub to form the hub, trimming the forging, then necking down the forging to shaft size to accomplish a 10 to 3-6 reduction immediately adjacent the hub, and forging by hammering down the forging to shaft size inwardly of the necking.

#### References Cited in the file of this patent

#### UNITED STATES PATENTS

|           |            |               |
|-----------|------------|---------------|
| 141,680   | Van Patten | Aug. 12, 1873 |
| 602,940   | Hall       | Apr. 26, 1896 |
| 1,325,067 | Wilcox     | Dec. 16, 1919 |
| 1,911,180 | Corlett    | May 30, 1933  |
| 2,027,980 | Horton     | Jan. 14, 1936 |
| 2,057,924 | Smith      | Oct. 20, 1936 |